

Feb. 24, 1942.

A. WESLEY ET AL

2,274,112

SEMIBRIGHT NICKEL DEPOSITION

Filed Dec. 29, 1938

3 Sheets-Sheet 1

Fig. 1.



Fig. 2.



INVENTORS

ANDREW WESLEY  
BY JAY WILLIAM CAREY  
A. Dr. Weller  
ATTORNEY

Feb. 24, 1942.

A. WESLEY ET AL

2,274,112

SEMIBRIGHT NICKEL DEPOSITION

Filed Dec. 29, 1938

3 Sheets-Sheet 2

Fig. 3.



Fig. 4.



INVENTORS

ANDREW WESLEY  
BY JAY WILLIAM CAREY  
A. P. O. Box 200  
ATTORNEY

Feb. 24, 1942.

A. WESLEY ET AL

2,274,112

SEMIBRIGHT NICKEL DEPOSITION

Filed Dec. 29, 1938

3 Sheets-Sheet 3

Fig. 5.



INVENTORS

ANDREW WESLEY  
BY JAY WILLIAM CAREY  
A. P. Weller  
ATTORNEY

## UNITED STATES PATENT OFFICE

2,274,112

## SEMIBRIGHT NICKEL DEPOSITION

Andrew Wesley, Plainfield, N. J., and Jay William Carey, Lynbrook, N. Y., assignors to The International Nickel Company, Inc., New York, N. Y., a corporation of Delaware

Application December 29, 1938, Serial No. 248,146

6 Claims. (Cl. 204—49)

The present invention relates to a process of producing semi-bright deposits of nickel, and more particularly to a process of producing semi-bright deposits of nickel by using an electroplating bath consisting principally or preferably substantially entirely of an aqueous solution of nickel chloride and boric acid in critical amounts under properly correlated critical conditions of temperature, current density and hydrogen ion concentration, and in the absence of "brightening addition agents."

Nickel deposits produced by ordinary commercial practice have been matte or dull in appearance, requiring expensive polishing and buffing operations to produce the desired bright appearance. In order to avoid the expense and disadvantages inherent in such prior art practice many attempts have been made to produce nickel coatings which were so smooth that no, or only slight, buffing was required to bring out a high luster. Coatings which gave a specular reflection without buffing were known in the art as "bright" whereas those which had the appearance of a mirrored surface that had been breathed upon and which required only slight buffing to produce a bright or mirror-like finish were designated "semi-bright" or "blushed." The art in recent years has attempted to produce bright and semi-bright deposits by the use of "brightening addition agents" in the electroplating bath. These agents were, generally speaking, additions of organic or inorganic materials such as sulfonated naphthalene or terpene compounds, albumins, cadmium salts and lead salts intended to give bright or semi-bright deposits directly in the bath. Even with the most recent improvements, this art suffered from several disadvantages which limited the commercial usefulness of baths containing brightening addition agents. The chief disadvantage was the difficulty of maintaining the bath composition constant over a period of time. The brightening addition agents were not perfectly stable and were difficult to maintain in constant concentration in the bath. So much highly skilled technical service had to be given to users of such baths that none of them was in widespread use in smaller plating shops. Other shortcomings of these processes were extreme brittleness of the deposit, a pronounced tendency for development of pits in the deposit and with some plating baths the permissible variation in plating conditions such as temperature and current density was very narrow.

Due to the difficulty of polishing and buffing ordinary matte electrodeposited nickel coatings

and of getting coatings of nickel free from pits, it was common practice to use multiple coatings of nickel and copper and to confine the polishing operations to the copper layer. Moreover, experts in the art advised against the use of a nickel chloride bath for depositing nickel directly on iron due to the poor bond formed between the coating and the iron which resulted in the plating peeling off a short time after deposition.

There was a definite and well recognized need in the art for a method of depositing single layer coatings of nickel free from pits and smooth enough to buff easily and which was not subject to the operating difficulties mentioned hereinabove.

We have invented a process of electrodepositing nickel free from pits and in such smooth form that a high luster can be developed by slight buffing. In our novel and improved process an easily controlled electroplating solution composed substantially entirely of an aqueous solution of nickel chloride and boric acid in critical amounts is used and the plating conditions including the hydrogen ion concentration, temperature and current density are controlled within critical limits properly correlated with the bath composition to produce satisfactory and acceptable semi-bright nickel deposits.

It is an object of the present invention to provide a process of producing semi-bright coatings of nickel which may be brought to a high luster with only slight buffing.

It is another object of the present invention to provide a process of producing semi-bright deposits of nickel by the use of a readily controllable electroplating bath capable of wide commercial use even in smaller plating shops where highly skilled technical service cannot practically be given.

It is a further object of the present invention to provide a process of producing semi-bright single layer coatings of nickel on other metals such as iron, steel, brass, etc., in which the plating conditions including hydrogen ion concentration, temperature and current density may be varied within relatively wide but critical limits by proper correlation with each other and with the bath composition.

The invention also contemplates a process of producing relatively thick coatings of electrodeposited nickel free from pits and excessive brittleness and which are so smooth that they may be brought to a high luster with slight buffing.

Other objects and advantages of the present invention will become apparent from the follow-

ing description taken in conjunction with the accompanying drawings in which:

Fig. 1 represents graphically the critical limits of the bath composition;

Figs. 2, 3 and 4 depict graphically the critical correlation between temperature and current density at pH values of 0.75, 1.0 and 2.0, respectively; and

Fig. 5 is a graph showing the results of a physical test for distinguishing between matte, semi-bright and bright deposits.

Generally speaking, the process of the present invention contemplates the electro-deposition of semi-bright nickel coatings on any appropriate foundation metal or alloy by the use of a plating bath containing principally nickel chloride and boric acid in aqueous solution without "brightening addition agents," and by properly correlating hydrogen ion concentration, current density and temperature within critical limits, as hereinafter described. The present invention makes it possible to produce directly thick deposits of semi-bright nickel so smooth that they require only slight buffing to be brought to a high luster. At the same time the deposits are satisfactory in respect to adherence, ductility, soundness and freedom from pits. The extreme simplicity of composition of the plating bath and the relatively wide range of permissible variation in plating conditions within critical limits make this process unusually easy to control. The process of the present invention, moreover, may be used to plate nickel directly on iron or steel, and the nickel plating so produced adheres well and has no tendency to peel off.

In the plating bath employed in the present invention, critical amounts of nickel chloride and boric acid are dissolved in water. Preferably the bath contains about 300 grams per liter of nickel chloride and about 30 grams per liter of boric acid. No addition of brightening agents of any kind need be made to the present improved bath to obtain the desired semi-bright nickel deposits. The boric acid content may vary from more than about 35 grams per liter down to less than about 5 grams per liter. Satisfactory results may be obtained provided more than a critical minimum content of boric acid is present which is designated by the curve A in Fig. 1. The abscissa in this graph represents boric acid concentration and the ordinate the nickel chloride concentration of the bath, both in grams per liter. If boric acid is present in an amount less than that depicted, the nickel deposit is burned and unsatisfactory. Beyond about 35 grams of boric acid per liter, the solubility of boric acid at room temperature is exceeded and flakes of boric acid settle out when the bath is allowed to cool. About 35 grams of boric acid per liter represents a practical maximum for commercial and industrial operations but the present invention is not limited to this amount as an absolute maximum. Satisfactory results may still be obtained when the boric acid concentration is substantially saturated at the operating temperature. While the theoretical function or functions of boric acid in its unique cooperation and combination with nickel chloride in the bath are not thoroughly understood, it is believed that boric acid does serve to buffer the solution. Curves B and C indicate minimum and maximum contents of nickel chloride in the form of  $\text{NiCl}_2 \cdot 6\text{H}_2\text{O}$ . Between the limits of about 260 grams and about 340 grams of  $\text{NiCl}_2 \cdot 6\text{H}_2\text{O}$  per liter satisfactory semi-bright deposits are ob-

tained. Either above or below these critical limits, matte deposits are formed. The curves in Fig. 1 were determined with a bath temperature of 100° F., a pH of 1.0 and a current density of 75 amperes per square foot, but the positions of the curves do not change substantially with varying plating conditions within the limits hereinafter set forth.

The acidity limits for producing satisfactory semi-bright deposits with the nickel chloride-boric acid bath are defined by about pH=0.7 and about pH=3.0. The pH is maintained by additions of hydrochloric acid instead of the customary sulfuric acid. These limits are critical. Numerous experiments have demonstrated that satisfactory semi-bright deposits cannot be obtained with the above mentioned bath unless the pH value is less than 3.0. Below a pH of about 0.7, the cathode current efficiency becomes too low for satisfactory commercial operation.

Bath temperature and current density must be coordinated with each other and with the hydrogen ion concentration in order to obtain the desired semi-bright deposit of nickel. These relationships are depicted graphically in Figs. 2, 3 and 4 in which the abscissa represents current density in amperes per square foot, and the ordinate is temperature in degrees Fahrenheit. The bath employed for each series of tests contained about 300 grams per liter of  $\text{NiCl}_2 \cdot 6\text{H}_2\text{O}$  and about 30 grams per liter of boric acid with the pH and other plating conditions controlled as hereinafter set forth.

In one series of tests, a constant pH of about 0.75 was maintained while current density and bath temperature were varied. Current densities from very low values to more than 200 amperes per square foot were found to produce satisfactory semi-bright nickel deposits provided the bath temperature did not rise above a critical value indicated by the curve D in Fig. 2. Below the curve D satisfactory semi-bright deposits were obtained, but above the curve the deposits were matte.

The pH value was maintained at about 1.0 for a second series of tests in which both temperature and current density were varied. Within the area defined by curves E and F in Fig. 3 satisfactory semi-bright deposits were produced. When the temperature lay above curve E at any particular current density the deposit was matte. Below curve F, the deposit is burned and unsatisfactory.

In Fig. 4, the results are plotted of a third series of tests conducted at a pH of about 2.0. The area between the curves G and H represents the conditions of temperature and current density which yield satisfactory semi-bright nickel deposits. Above curve G and below curve H the deposits are matte and burned respectively as described in connection with Fig. 3.

It will be seen from a study of Figs. 2, 3 and 4 that the area defining the ranges of permissible temperatures and current densities decreases progressively as the pH rises. A fourth series of tests conducted at pH=3.0 demonstrated that the area had substantially disappeared. While the operable range of pH is about 0.7 to about 3.0, practical limits for semi-bright plating on a commercial scale are about pH=0.75 and about pH=2.0. Temperatures from about 80° F. to about 145° F. are satisfactory for commercial operation with current densities varying from about 20 to about 200 amperes per square foot. Current density, temperature and pH should

preferably be so correlated as to fall well within the semi-bright areas of Figs. 2, 3 and 4.

It will be understood by those skilled in the art that lines of curves D, E, F, G and H actually represent areas of somewhat varying width. In other words, for any given current density and pH, e. g., 140 amperes per square foot and pH=1, the deposit does not suddenly change from semi-bright to matte with a slight temperature change, e. g., from slightly less to slightly more than 141° F. (see Fig. 3). On the contrary, there is a relatively narrow temperature range over which the deposit changes rather rapidly from semi-bright to matte.

The following specific example is illustrative of the results that may be obtained by practicing the present invention.

An aqueous plating bath was prepared having the following composition:

NiCl<sub>2</sub>·6H<sub>2</sub>O about 300 grams per liter  
H<sub>3</sub>BO<sub>3</sub> about 30 grams per liter

Sufficient hydrochloric acid was added to the aqueous solution to adjust the pH to about 1.0.

A bagged, rolled, depolarized nickel anode was used and the solution was filtered continuously. Slight agitation of the bath was obtained by means of a gentle stream of air. The bath temperature was maintained at about 110° F. while a steel object was coated directly with nickel at a cathode current density of about 75 amperes per square foot. After about 19 minutes a semi-bright deposit about 0.001 inch thick had been formed which was brought to a high finish in a single buffering operation using a soft rag wheel treated with an ordinary grease coloring compound containing rouge. A bright, mirror-like surface was obtained at a given point in about 10 seconds.

The art recognizes three general classes of nickel plating, viz., the ordinary white nickel, bright nickel and semi-bright or blushed nickel. The term "white" nickel has been used to describe the color of matte deposits and has no reference to any degree of brightness. A "bright" deposit is one which gives a specular reflection of incident light and is mirror-like in appearance. Images of objects seen in a flat surface coated with bright nickel appear clear and distinct. A "dull" or "matte" deposit is one which reflects so little light specularly that no images can be distinguished in a flat surface coated with matte nickel except at grazing angles of incidence. Instead of specular, there is diffuse reflection. A "semi-bright" deposit is one approaching the smoothness of a bright deposit but falling somewhat short of a specular reflection of incident light. It appears like a mirror that has just been lightly breathed on. The terms "blushed" and "milky" are also used to describe semi-bright deposits. Enough light is reflected specularly that images of objects can be distinguished at fairly small angles of incidence, albeit not very clearly and with hazy, instead of sharp, edges.

In order to define more precisely the difference between matte, semi-bright and bright deposits, results of brightness measurements made by the method originated by P. Bouger [Traité d'Optique sur la Gradation de la Lumière, Paris, Guerin and Delatour (1760)] have been plotted in Fig. 5. In performing these measurements, the specimen, in the form of a flat rectangular piece of steel sheet coated with a nickel deposit about 0.001 inch thick, was placed at the center of a

spectrometer table and in a plane normal to the table. It was illuminated by a thin collimated beam of white light of about 1500 foot candles intensity, incident upon the specimen at a known angle with respect to the surface of the specimen. The light emitted directly back from the specimen was then reflected from the surface of a thin cover glass, placed at 45° to its path, toward an illuminometer which was used to measure the intensity of the reflected beam in apparent foot candles. By inclining the specimen at various angles to the incident beam, data for curves correlating the angle of incidence (which in this procedure is the same as the angle of reflection) and the intensity of the reflected light was obtained.

These data for typical matte, semi-bright and bright specimens with coatings 0.001 inch thick are plotted in curves I, J and K of Figure 5 which involve quite different magnitudes and distributions of intensities for the different types of deposit. Almost all of the light reflected from a truly bright nickel deposit is reflected in one direction and the maximum intensity observed is at least about 50% or more of the intensity of the incident light. (See curve K.) Typical semi-bright or blushed deposits are characterized by one or more peaks in the curve with a maximum observed intensity within the range of about 30 to about 600 foot candles when the incident light has an intensity of about 1500 foot candles, i. e., the reflected light is about 2 to 40% of the incident light. (See curve J.) Typical matte deposits, however, reflect light of less than 20 foot candles intensity under comparable conditions over a wide range of angles of incidence and reflection, i. e., about 1.5% or less. (See curve I.)

It will be apparent from the foregoing that the present invention provides a practicable and satisfactory process of producing semi-bright nickel deposits. The bath is relatively inexpensive, easy to make up and maintain, and is stable. For example, a bath of the type described hereinbefore has been operated for the purposes of testing over a period of years depositing semi-bright nickel on a great number of steel test pieces during that time. At the end of the period, the bath produced just as good semi-bright nickel deposits as at the beginning. Although the nickel was deposited directly on the steel foundation metal, it adhered strongly thereto and did not peel off even when exposed for long periods to the atmosphere. Slight buffering, for example, with a rag buffering wheel and ordinary rouge buffering compound for about 10 seconds, produced a bright, mirror-like finish at any particular spot. Deposits as thick as about 0.006 inch may readily be obtained by the process embodying our invention which are still semi-bright and readily polished with slight buffering to bright, mirror-like finish.

We claim:

1. A plating bath consisting of an aqueous solution containing nickel chloride within the range of about 230 to about 340 grams per liter, boric acid from about 2 grams per liter to saturation at the bath operating temperature, and sufficient hydrochloric acid to regulate the pH between about 0.7 and 3.0.

2. A process of electrodepositing adherent, semi-bright coatings of nickel on a foundation metal comprising establishing an aqueous plating bath consisting principally of about 260 to 340 grams per liter of nickel chloride and from about 2 grams to about 35 grams per liter of boric acid, adjusting the pH value of the bath between about

0.7 and less than 3 by additions of hydrochloric acid, heating the bath to a temperature of about 80° F. to about 145° F., and depositing nickel upon a foundation metal at a current density of about 20 to about 200 amperes per square foot to produce a semi-bright adherent coating of electro-deposited nickel on the foundation metal.

3. A process of electrodepositing adherent, semi-bright coatings of nickel on a foundation metal comprising establishing an aqueous plating bath consisting principally of about 260 to 340 grams per liter of nickel chloride and from about 2 grams to about 35 grams per liter of boric acid, adjusting the pH value of the bath between about 0.7 and less than 3 by additions of hydrochloric acid, heating the bath to a temperature of about 80° to 145° F., making a piece of foundation metal to be plated a cathode in said bath, and depositing nickel thereon at a current density within the semi-bright areas represented by the curves of Figures 2, 3 and 4 for the particular temperature of the bath.

4. A plating bath consisting of an aqueous solution containing about 300 grams of nickel chloride per liter, about 30 grams of boric acid per

liter and sufficient hydrochloric acid to regulate the pH between about 0.7 and about 3.0

5. An aqueous nickel electropating bath consisting principally of an aqueous solution of about 260 to about 340 grams of nickel chloride per liter, about 5 to about 35 grams of boric acid per liter and sufficient hydrochloric acid to provide a pH of about 0.7 to about 3.0.

6. A process for depositing adherent electro-deposits of nickel directly upon a ferrous base metal which comprises electro-depositing nickel from an aqueous plating bath consisting principally of about 260 to about 340 grams per liter of nickel chloride and from about 5 grams to about 35 grams per liter of boric acid, adjusting the pH value of the bath between about 0.7 and less than 3 by additions of hydrochloric acid, heating the bath to a temperature of about 80° F. to about 145° F. and depositing nickel upon said ferrous base metal at a current density of about 20 to about 240 amperes per square foot to produce a semi-bright adherent coating of electro-deposited nickel on the aforesaid ferrous base metal.

ANDREW WESLEY.  
JAY WILLIAM CAREY.